

# United States Patent

Pfeiffer et al.

[15] 3,645,121

[45] Feb. 29, 1972

[54] **METHOD FOR ROLLING TUBULAR MATERIAL STOCK IN A STRETCH REDUCING MILL**

[72] Inventors: Gerd Pfeiffer; Horst Biller, both of Mulheim-Ruhr; Claus Schrey, Oberhausen; Alfred Schmitz, Mulheim-Ruhr, all of Germany

[73] Assignee: Mannesmannrohren-Werke GmbH, Dusseldorf, Germany

[22] Filed: July 1, 1969

[21] Appl. No.: 838,384

[30] **Foreign Application Priority Data**

July 5, 1968 Germany .....P 17 52 713.8

[52] U.S. Cl.....72/205, 72/208, 72/367,  
72/234

[51] Int. Cl.....B21b 17/00

[58] Field of Search .....72/205, 234, 249, 208

[56]

**References Cited**

**UNITED STATES PATENTS**

|           |         |                   |          |
|-----------|---------|-------------------|----------|
| 2,342,767 | 2/1944  | Stoltz.....       | 72/234 X |
| 3,036,480 | 5/1962  | Schwab.....       | 72/11 X  |
| 3,151,508 | 10/1964 | Holman et al..... | 72/234 X |
| 3,308,644 | 3/1967  | Voin Dorp.....    | 72/249   |

*Primary Examiner*—Milton S. Mehr  
*Attorney*—Burgess, Dinklage & Sprung

[57]

**ABSTRACT**

A method for rolling down tubular material in a rolling mill wherein in the vicinity of the starting sections and/or end sections of the tubular material normally having thickened portions a stepwise variation of the rotational speeds is provided at the roll stands deforming these sections, said stepwise variation of said rotational speeds required for rolling the central section of the tubular material.

7 Claims, 8 Drawing Figures

PATENTED FEB 29 1972

3,645,121

SHEET 1 OF 6



Inventors:  
Gerd Pfeiffer, Horst Biller,  
Claus Schrey, and Alfred  
Schmitz  
By: Burges, Dicklegg & Speng  
Attorneys

Fig. 3



Inventors:

Gerd Pfeiffer, Horst Biller, Claus Schrey  
and Alfred SchmitzBy: Burgher, Dinklage & Sprung  
Attorneys

Fig. 5

PRIOR ART



Fig. 4

PRIOR ART



## Inventors:

Gerd Pfeiffer, Horst Biller, Claus  
Schrey and Alfred Schmitz

By: Burgen, Dinklage & Sprung  
Attorneys

Fig. 6



Inventors:  
 Gerd Pfeiffer, Horst Biller, Claus  
 Schrey, and Alfred Schmitz  
 By: Burgers, Den Blaag & Sprung  
 Attorneys

Fig. 7



Inventors:  
 Gerd Pfeiffer, Horst Biller, Claus  
 Schrey, and Alfried Schmitz  
 By: Burges, Dinklage & Sprung  
 Attorneys

Fig. 8



Inventors:  
 Gerd Pfeiffer, Horst Biller, Claus  
 Schrey, and Alfred Schmitz  
 By: Burgers, Dinklage & Sprung  
 Attorneys

METHOD FOR ROLLING TUBULAR MATERIAL STOCK  
IN A STRETCH REDUCING MILL

Tubular material is reduced in its diameter in a rolling mill without an internal die in a plurality of consecutive stand locations. In addition to this diameter reduction generally, a change in the wall thickness is also effected, the rate of which depends on the stress condition existing in the rolled product. The stress condition in the rolled product which can be defined by the "related longitudinal tension"

$$X_L = (K_L/F \cdot k_f)$$

( $K_L$  = the longitudinal force acting on the tubular cross section,

$F$  = tubular cross section,

$k_f$  = the mean tensile strength of the material of the rolled product),

is influenced by the stepwise change in the rotational speeds of the individual stand locations. The more the longitudinal tension  $X_L$  is influenced by the stepwise change in the rotational speeds, the thinner the wall of the reduced tubular material will be. In order to thus obtain a desired wall thickness, a predetermined rotational speed sequence must be set in the rolling mill which yields the longitudinal tension required at the individual stand locations.

In conventional methods for rolling down tubular material the longitudinal tension at the beginning and at the end of the tubular material does not nonsequentially rise and fall between zero and the predetermined rate with the preset rotational speed sequence, but stepwise. A tension rise as per definition is present in a stand in the event that the longitudinal tension between the stand location  $m+1$  and the stand location  $m$  is greater than the longitudinal tension between the stand location  $m$  and the stand location  $m-1$ . A tension fall is present in a stand location  $k$  in the event that the longitudinal tension between the stand location  $k+1$  and the stand location  $k$  is smaller than the longitudinal tension between the stand location  $k$  and the stand location  $k-1$ . At the initial section of the tubular material the longitudinal tension thus is decreased, whereas at the rearward section of the tubular material entering the first stand locations the longitudinal tension is increased. It follows therefrom that the forward section and the rearward section of the tubular material to be reduced are subjected to a lower longitudinal tension than required for the desired wall thickness variation. The predetermined rating of the longitudinal tension and thus the desired wall thickness variation is achieved in the central portion of the tubular material only. The front end and the rear end of the tubular material are thickened tubular pieces and are cut off as waste, a necessary result of the method.

It is an object of the invention to provide a method for rolling down tubular material in a rolling mill wherein the thickened front section of the tubular material is substantially shortened at least as compared with the front section of the tubular material thickened in the conventional methods.

A further object of the invention is to also substantially shorten the thickened rear section of the tubular material at least as compared with the thickened rear section of the tubular material obtained by the prior art methods.

According to this invention, a stepwise variation of the rotational speeds is provided for rolling down tubular material in a rolling mill in the vicinity of the front sections and/or rear sections of the tubular material normally having thickened portions at the stands deforming these sections, said stepwise variation of the rotational speeds being greater than the stepwise variation of the rotational speeds required for rolling the central section of the tubular material.

This method is conveniently provided such that as far as the front section of the tubular material is concerned, the rotational speeds of the rolls at a plurality of stand locations 1 through  $m$  are decreased prior to the entry of the front section of the tubular material relative to the rotational speed sequence when the rolling mill is filled, the percentage in the rotational speed decrease being greatest at the first stand location and decreasing with the increasing number of the stand location, and that then when the front section of the tubular

material enters the reducing rolling mill the decreased rotational speeds of the individual stand locations are increased again dependent on the passing of the front section of the tubular material through a plurality of stand locations to the speed sequence with filled rolling material. The increase of the decreased rotational speeds can be effected in increments or continuously at the stand locations which the front section has passed.

This invention furthermore contemplates that the percentage in the increase of the rotational speeds to the rotational speeds with filled rolling mill is effected uniformly at all stand locations through which the front section of the tubular material passes. The rotational speeds of the stands through which the front section of the tubular material passes can be respectively increased in such a manner that they receive the same percentage in the rotational speed decrease as the ultimate stand location rolling the front end of the tubular material.

Since the speed differentials of the stand locations effective as tension diminishing upon entry of the front section of the tubular material are greater by the rotational speed decrease than later upon rolling the central section of the tubular material where the stand locations are effective as stand locations maintaining the tension constant, the thickened front section of the tubular material can be greatly shortened. The speed differentials can even be selected sufficiently large so that there is no point on the pressed surface of the caliber having the same speed as the tubular material. In this case the roll slides in all contacting points on the tubular material due to its higher circumferential speed of the caliber relative to the tubular material. By increasing the speed differentials for rolls already slipping by an increase of the frictional work applied to the tubular material the longitudinal tension in the tension decreasing stands can be increased to a predetermined limit which can be determined by tests.

The method according to the invention will be discussed in greater detail hereinafter, for the front section of the tubular material, with reference to the accompanying drawings.

FIG. 1 is a diagrammatic illustration of a rolling mill with the tubular material entering, said rolling mill being operated according to conventional practice, the longitudinal tension occurring in the tubular material being indicated;

FIG. 2 an illustration similar to FIG. 1 of the rolling mill illustrated there with the tubular material having passed further into the rolling mill;

FIG. 3 an illustration of the rotational speed decrease and rotational speed increase at the individual stand locations or a rolling mill operating according to the method of this invention.

FIG. 4 is a diagrammatic illustration of a rolling mill operated in accordance with the conventional method in the filled state with the longitudinal tension existing in the tubular material;

FIG. 5 is a diagrammatic illustration of the rolling mill illustrated in FIG. 4 with outgoing tubular material, the longitudinal tension existing in the tubular material being illustrated;

FIG. 6 is an illustration of the speed reduction and speed increase in the individual stand locations of a rolling mill in accordance with the method of this invention;

FIG. 7 is an illustration of the speed reduction in the individual stand locations of a rolling mill in accordance with a variant of the method of this invention.

In the rolling mill illustrated in FIG. 1 the tension increase is effected in the stand locations 1 and 2, whereas the tension decrease is effected in the stand locations 5 and 6 for the rotational speed sequence set. The longitudinal tension is constant between the stand locations 2 and 3 on the one side and the stand locations 3 and 4 on the other side. The stand location 3 located in the central tubular section thus is a stand location maintaining the tension constant.

As illustrated in FIG. 2 the tension decrease has shifted with the advancing of the front section of the tubular material from the stand locations 5, 6 via the stand locations 6, 7 to the stand

locations 7, 8. The stand locations 5, 6 have turned into stand locations maintaining the tension constant with unaltered rotational speeds.

Since in the conventional method the front section of the tubular material is rolled with a longitudinal tension during the entire passing through the stand, said longitudinal tension being below the longitudinal tension required for the desired wall thickness, the wall thickness of the front section of the tubular material is thicker than the wall thickness of the central section of the tubular material. The length of the thickened front section of the tubular material depends on the number of the stand locations which are required for the stepwise tension decrease. In FIGS. 1 and 2 the length of the front section is at least equal to the spacing of two adjacent stand locations.

In order to substantially shorten this thickened front section, according to this invention the rotational speeds of the individual stand locations are decreased prior to the entry of the tubular material, as is illustrated in FIG. 3. In the drawing 11 stand locations are illustrated. The percentage in the rotational speed decrease from the entry of the tubular material relative to the rotational speed with a filled rolling mill amounts to 5 percent between the individual stand locations, so that rotational speed decrease of the stand location 1 is 50 percent, that of stand location 2 is 45 percent etc., and finally that of stand location 11 is 0 percent. The increments in the decrease and the number  $m$  of the stand locations with decreased speed is dependent on the minimum and maximum rating of the longitudinal tension required for shortening the thickened front section of the tubular material and of the control range of the motors of the stand locations, in particular of the first stand location, i.e., the stand location number must be selected such that for a predetermined stepwise variation of the speed decrease the speed decrease of the first stand location is within the control range of the coupled motor or engine. When specifying the stepwise variation of the rotational speeds between the adjacent stands it must be observed that it is not selected at too large a value because otherwise a tearing off of the tubular material is effected.

When the tubular material now enters the rolling mill, an increased longitudinal tension is exerted on the front section due to the percentage in the stepwise speed reduction at the stand locations 1 to 11. This front section of the tubular material has been illustrated in FIG. 3 as a full drawn beam.

In phase I the front section extends across the stand locations 1 to 5 with the speed reduction in increments of respectively 5 percent from 50 percent at stand location 1 to 30 percent at the stand location 5. In phase II the front section of the tubular material has passed stand location 1. The speed reduction of stand location 1 has been raised to the speed reduction of stand location 2. In phase III the front section of the tubular material has passed through stand location 2, the speed reduction of which is increased together with the speed reduction of stand location 1 to the speed reduction of stand location 3, namely to 40 percent. With the front section of the tubular material further advancing the speed reductions are increased in an according manner in phases IV to X, so that finally in phase XI all stand locations have been increased to the speeds of the filled rolling mill. In the diagrammatic illustration of the individual phases it will be noted that the central section of the tubular material is not subjected to any increased tension during the speed increase, since the stands rolling the central section of the tubular material are not operated relative to one another with speeds of unequal increments in their percentage relative to the speeds with the rolling mill filled, but with rotational speeds of equal increments in their percentage.

The problem of substantially shortening the thickened section of the tubular material for the rear sections of the tubular material is conveniently solved in the following manner, there being two possibilities:

In the first of these possibilities the problem is solved in that with the rolling mill filled, the roll speed of all stands ( $p$  in number) participating in the deformation of the tubular material are reduced relative to the speed sequence used for

rolling the central section of the tubular material, the percentage in the speed reduction at all stands being equal; thereafter when the rear section of the tubular material enters the sequence of stands 1 through  $n$  of the rolling mill the reduced speeds of the stands 2 through  $p$  are increased dependent on the passing of the rear section of the tubular material through the stands 1 through  $n$  in such a manner that the percentage in the speed reduction in the vicinity of the rear section of the tubular material decreases with an increasing number of stand locations to the stand  $n$ , and that the central section of the tubular material is rolled in stands the percentage of speed reduction of which is equal.

Stands 1 thus maintains the overall reduction; stand 2 is increased only once in the speed; stand 3 is increased in the speed twice etc., up to the stands  $n$  through  $p$  which are increased  $n$  minus once and thereby reach the initial speeds again. The decrease and increase of the speeds can be effected continuously or in increments. The number  $n$  of the sequence of stands in which the rolling speeds are reduced can be determined on the basis of tests.

A feature of the invention contemplates that the percentage increase of the rotational speeds of the stands which roll the central section of the tubular material is effected uniformly. This invention furthermore contemplates that the rotational speeds at the stand locations 1 through  $n$  are maintained after the rear section of the tubular material has left the rolling mill for the initially described method for shortening the thickened front section of the tubular material.

Since the speed differentials of the stand locations operating tension increasing upon entry of the rear section of the tubular material are greater by the speed reduction than when rolling the central portion of the tubular material when the stand locations are operating as stand locations maintaining the tension constant, the thickened rear section of the tubular material can be greatly shortened. The rotational speed differentials can even be selected sufficiently large so that there is no point on the pressed surface of the caliber which has the same speed. In this case the roll slips in all contacting points on the tubular material as a result of its circumferential speed lower relative to the tubular material. By increasing the speed differentials for rolls already slipping the longitudinal tension can be increased in the tension decreasing stands by increasing the frictional work applied to the tubular material within a predetermined limit determined by tests.

This method is explained in greater detail hereinafter in referring to FIGS. 3 to 6.

In the rolling mill illustrated in FIG. 4 the tension buildup is effected in stand locations 1 and 2, whereas the tension decrease is effected in stand locations 7 and 8 for the preset rotational speed sequence. The longitudinal tension is constant between stand locations 5 and 6 on the one side and stand locations 6 and 7 on the other side. Stand location 6 disposed in the central section of the tubular material thus is a stand location maintaining constant tension.

As illustrated in FIG. 5, the tension buildup has varied with the tubular material leaving the mill as compared to the condition with the mill filled, so that not the stand locations 1 and 2, but the stand locations 3 and 4 are stand locations building up tension.

Since in the prior art methods the rear section of the tubular material is rolled with a longitudinal tension during the entire passing through the stand, said longitudinal tension being below the longitudinal tension required for the rolled wall thickness, the wall thickness of the rear section of the tubular material will be thicker than the wall thickness of the central section of the tubular material. The length of the thickened rear section of the tubular material depends on the number of stand locations which is required for the incremental tension built up. In FIG. 4 and 5 the length of the rear section is at least equal to the spacing of two adjacent stand locations.

In order to now substantially shorten this thickened rear section, according to a feature of this invention the rotational speeds of the individual stand locations are reduced prior to

entry of the rear section of the tubular material, starting from the rotational speed sequence for the deformation of the central section of the tubular material, as illustrated in FIG. 6. In the drawings, 24 stand locations have been illustrated. The amount of the reduction depends on the minimum and maximum rating of the longitudinal tension required for the shortening of the thickened rear section of the tubular material, of the diameter reduction sequence employed (increments of the diameter reduction from one stand to the other), and of the control range of the motors or engines of the stand locations.

In the drawings the percentage rotational speed reduction has been selected with 50 percent for all 24 stands prior to entry of the rear section of the tubular material into the rolling mill. Upon entry of the rear section of the tubular material into the first stand the rotational speeds are increased by 5 percent from stand 2 to 24, i.e., a tubular section results between stand 1 and 2 which is subjected to an increased longitudinal tension of the differential of the rotational speeds of 50 percent minus 45 percent, or 5 percent. The exact time the rotational speed is increased is determined by the length of the rear section of the tubular material which has not yet entered the rolling mill, which will normally be 1 to 5 stand spacings, in considering the time required for balancing the speed increase. In the drawing this length is 3 stand spacings. Upon entry of the rear section of the tubular material in the second stand the rotational speeds are increased by 5 percent from stand 3 to stand 24, again the time required for balancing the speed increase having to be considered so that the speed reduction amounts to 40 percent for these stands, whereas it amounts to 45 percent for the second stand and 50 percent for the first stand. In FIG. 6 the rear section of the tubular material on which an increased longitudinal tension is exerted is characterized as a beam drawn in full lines. In phase I the longitudinal section subject to an increased longitudinal tension extends from stand 1 to 2, the stands 2 to 24 having a speed reduction of 45 percent and stand 1 having a speed reduction of 50 percent. In the phase II stand 1 is reduced in its speed by 50 percent, stand 2 by 45 percent and stands 3 to 24 by 40 percent. With further advancing rear section of the tubular material the speed reduction is accordingly cancelled until in phase XIII the stand locations 11 to 24 have been stepped up to the normal speed again. The quoted percentages have been selected only for a better understanding in the given magnitude. The ratings suitable for performing the invention can be determined such that they are precalculated by means of the factors decisive for the amount of the speed reduction such as longitudinal tension required, diameter reduction sequence, control range of the motors or engines, which are then checked by test rolling and are corrected. It will be noted from the diagrammatic illustration that the central section of the tubular material is not subjected to any increased tension for reduced speeds, since the stands rolling the central section of the tubular material are reduced by the same percentage in their speed, i.e., that the ratio of the speeds for stands which roll the central portion of the tubular material

(for instance  $\frac{\text{speed for stand 8}}{\text{speed for stand 9}}$  in phase V).

for the reduced condition is equal to the ratio of the speeds in the nonreduced condition.

FIG. 6 discloses that after the rear section of the tubular material has left the rolling mill the speed reductions still present at the stand locations 1 to 11 according to phase XIII are identical to phase I according to FIG. 3 which illustrates the speed reduction in the individual stand locations of a rolling mill for shortening the thickened front section of the tubular material. It will be noted therefrom that the method of this invention permits the performing of the method for shortening the thickened front section of the tubular material for the following tube or pipe without any particular preparation.

In the second of these possibilities the problem is solved in that upon entry of the rear section of the tubular material in

consecutive stands 1 through  $q$  the associated roll speeds thereof are reduced dependent on the passing of the rear section of the tubular material through these stands such that in the vicinity of the rear section of the tubular material the percentage in the speed reduction decreases with increasing stand location number, and that the central section of the tubular material is rolled in stands with unaltered rotational speed. The reduction of the rotational speeds can be effected continuously or in increments. The rotational speeds of the stands which just roll the rear section of the tubular material are at the same time reduced. The number  $q$  of the consecutive stands in which the roll rotational speeds are reduced can be determined on the basis of tests.

This invention furthermore contemplates that the percentage in the rotational speed reduction of the stand group respectively rolling the rear section of the tubular material is effected uniformly.

Since the rotational speed differentials of the stand locations operating tension increasing upon entry of the rear section of the tubular material are greater by the speed reduction than when rolling the central portion of the tubular material when the stand locations operate as stand locations maintaining constant tension, the thickened rear section of the tubular material can be greatly shortened.

The amount of the reduction depends on the minimum and maximum rating of the longitudinal tension required for shortening the thickened rear section of the tubular material, on the diameter reduction sequence employed (increments of the diameter reduction from one stand to the other), and on the control range of the engines or motors of the stand locations.

This method will be explained in closer detail hereinafter in referring to FIG. 7 of the accompanying drawings:

In FIG. 7, nine stand locations have been illustrated of a rolling mill. Starting from the rotational speed sequence for the deformation of the central portion of the tubular material the associated speed is reduced by 5 percent in stand 1 upon entry of the rear section of the tubular material, the speed relationship for the speed of the stands 1 and 2 thereby being varied such that the longitudinal tension existing in the tube or pipe is increased in (phase I). The exact point at which the rotational speed is reduced is determined by the length of the rear section of the tube or pipe which has not yet entered the rolling mill, which is normally between one and five stand spacings, in considering the time required for balancing the speed reduction; in the drawing this length is two stand spacings.

Upon entry of the rear section of the tubular material into the second stand the rotational speeds are reduced from stand 1 and 2 by 5 percent, again the time required for balancing the rotational speed reduction having to be considered. In phase II the speed reduction for the first stand is 10 percent and for the second stand 5 percent. Thereby an increased longitudinal tension results in a tubular section extending from stand one to stand 3. When the rear section of the tubular material advances further through the rolling mill, the rotational speed reduction is accordingly repeated in such a manner that the respectively last stand in the stand group rolling the rear section of the tubular material is subjected to the maximum speed reduction, for instance 15 percent for stand 5 in phase VII, and the first stand of the stand group is subjected to the minimum reduction, for instance 5 percent for stand 7 in phase VII. In FIG. 7 the rear section of the tubular material on

which an increased longitudinal tension is exerted is characterized respectively as a beam drawn in full lines in the individual phases. The cited percentages have been selected merely for a better understanding in the instant magnitude. The ratings suitable for performing the invention can be determined such that they are first precalculated by means of the practice decisive for the amount of the speed reduction, such as longitudinal tension required, diameter, reduction sequence, control range of the motors and engines, which are then checked by test rolling and are corrected. After the tube or pipe leaves the stands of the rolling mill, the rotational

speeds for the stands which have been subjected to a speed reduction are returned to those ratings for which they were set prior to the speed reduction for rolling the central section of the tubular material.

Naturally, the invention is in no way limited to the manners of carrying it out described herein by way of example. Variations may be resorted to, insofar as these changes come within the scope of the following claims.

What is claimed is:

1. A method of rolling down tubular material in a rolling mill in which the rolls of consecutive stands normally operate gradually increasing rotational speed, which comprises:

a stepwise reduction of the rotational roll speeds at a plurality of roll stands prior to entry of the front section of the tubular material, the percentage of the rotational speed reduction being at a maximum at the first stand location and decreasing at the subsequent stands; and subsequently, upon entry of the front section of the tubular material into the rolling mill, an increase in speed of the individual stand locations, dependent on the passing of such front section through a plurality of stand locations, to the rotational speed sequence for a filled rolling mill, so that the normally thickened front section of the tubular material is substantially shortened.

2. A method as defined in claim 1, wherein the percentage increase of the rotational speeds to the rotational speeds for the filled rolling mill is effected uniformly at all stand locations through which the front section of the tubular material passes.

3. A method as defined in claim 2, wherein the rotational speeds of the stand locations through which the front section of the tubular material passes are respectively increased such that they attain the same percentage speed reduction as the last stand location rolling the front section of the tubular material.

4. A method of rolling down tubular material in a rolling mill in which the rolls of consecutive stands normally operate

with gradually increasing rotational speed, wherein with the rolling mill filled the roll speeds of all stands,  $p$  in number, participating in the deformation of the tubular material are reduced relative to the speed sequence employed for rolling

5 the central section of the tubular material, the percentage rotational speed reduction at all stands being equal, and wherein subsequently upon entry of the rear section of the tubular material is consecutive stands 1 through  $n$  of the rolling mill the reduced speeds of the stands 2 through  $p$  are increased

10 dependent on the passing of the rear section of the tubular material through the stands 1 through  $n$  such that in the vicinity of the rear section of the tubular material the percentage rotational speed reduction decreases with an increasing stand location number up to the stand location  $n$ , and wherein the

15 central section of the tubular material is rolled in stands the percentage rotational speed reduction of which is equal.

5. A method as defined in claim 4, wherein the percentage increase of the rotational speeds of the stands which roll the central section of the tubular material is effected uniformly.

20 6. A method of rolling down tubular material in a rolling mill in which the rolls of consecutive stands normally operate with gradually increasing rotational speed, wherein upon entry of the rear section of the tubular material in consecutive stands 1 through  $q$  the associated roll rotational speeds thereof

25 are reduced dependent on the passing of the rear section of the tubular material through these stands such that in the vicinity of the rear section of the tubular material the percentage rotational speed reduction decreases with an increasing stand location number and wherein the central section of the

30 tubular material is rolled in stands with unaltered rotational speeds.

7. A method as defined in claim 6, wherein the percentage rotational speed reduction of the stand group respectively rolling the rear section of the tubular material is effected

35 uniformly.

\* \* \* \* \*

40

45

50

55

60

65

70

75

UNITED STATES PATENT OFFICE  
CERTIFICATE OF CORRECTION

Patent No. 3,645,121

Dated Feb. 29, 1972

Inventor(s) Gerd Pfeiffer et al.

It is certified that error appears in the above-identified patent and that said Letters Patent are hereby corrected as shown below:

In the Drawings: Cancel Figure 7 and renumber Figure 8 as Figure 7.

Signed and sealed this 13th day of June 1972.

(SEAL)

Attest:

EDWARD M. FLETCHER, JR.  
Attesting Officer

ROBERT GOTTSCHALK  
Commissioner of Patents

UNITED STATES PATENT AND TRADEMARK OFFICE  
CERTIFICATE OF CORRECTION

PATENT NO. : 3,645,121

DATED : February 29, 1972

INVENTOR(S) : Gerd Pfeiffer and Horst Biller

It is certified that error appears in the above-identified patent and that said Letters Patent is hereby corrected as shown below:

The title page, add the following to [30] Foreign Application  
Priority Data:

-- May 31, 1969 Germany 19 27 879

May 31, 1969 Germany 19 27 880

Signed and Sealed this

Seventeenth Day of February 1981

[SEAL]

Attest:

RENE D. TEGTMEYER

Attesting Officer

Acting Commissioner of Patents and Trademarks